



US010443013B2

(12) **United States Patent**  
**Ugamura et al.**

(10) **Patent No.:** **US 10,443,013 B2**  
(45) **Date of Patent:** **Oct. 15, 2019**

(54) **VISCOSITY INDEX IMPROVER, METHOD FOR PRODUCING THE SAME AND LUBRICATING OIL COMPOSITION**

USPC ..... 508/291, 469  
See application file for complete search history.

(71) Applicant: **NIPPON SHOKUBAI CO., LTD.**,  
Osaka (JP)

(72) Inventors: **Tadayoshi Ugamura**, Osaka (JP);  
**Kazunari Yasumura**, Osaka (JP);  
**Keiko Izumi**, Osaka (JP)

(73) Assignee: **NIPPON SHOKUBAI CO., LTD.**,  
Osaka (JP)

(\*) Notice: Subject to any disclaimer, the term of this  
patent is extended or adjusted under 35  
U.S.C. 154(b) by 32 days.

(21) Appl. No.: **15/503,032**

(22) PCT Filed: **Sep. 15, 2015**

(86) PCT No.: **PCT/JP2015/076181**

§ 371 (c)(1),

(2) Date: **Feb. 10, 2017**

(87) PCT Pub. No.: **WO2016/043195**

PCT Pub. Date: **Mar. 24, 2016**

(65) **Prior Publication Data**

US 2017/0233675 A1 Aug. 17, 2017

(30) **Foreign Application Priority Data**

Sep. 17, 2014 (JP) ..... 2014-189053  
Apr. 8, 2015 (JP) ..... 2015-079392

(51) **Int. Cl.**

*C10L 1/22* (2006.01)  
*C10M 145/14* (2006.01)  
*C10M 149/10* (2006.01)  
*C10M 149/06* (2006.01)  
*C10M 177/00* (2006.01)

(52) **U.S. Cl.**

CPC ..... *C10M 149/10* (2013.01); *C10M 149/06* (2013.01); *C10M 177/00* (2013.01); *C10M 2209/084* (2013.01); *C10M 2217/028* (2013.01); *C10N 2220/021* (2013.01); *C10N 2220/022* (2013.01); *C10N 2230/02* (2013.01); *C10N 2230/68* (2013.01); *C10N 2240/10* (2013.01); *C10N 2270/00* (2013.01)

(58) **Field of Classification Search**

CPC ..... C10M 2209/084; C10M 145/14

(56)

**References Cited**

**U.S. PATENT DOCUMENTS**

|                  |         |               |                    |
|------------------|---------|---------------|--------------------|
| 2010/0167970 A1* | 7/2010  | Stoehr        | ..... B01F 17/0028 |
|                  |         |               | 508/469            |
| 2014/0135243 A1  | 5/2014  | Takagi et al. |                    |
| 2014/0315771 A1  | 10/2014 | Iwai          |                    |
| 2015/0175926 A1  | 6/2015  | Matsui et al. |                    |
| 2015/0184109 A1  | 7/2015  | Matsui et al. |                    |
| 2015/0197705 A1  | 7/2015  | Matsui et al. |                    |
| 2015/0203781 A1  | 7/2015  | Matsui et al. |                    |
| 2015/0203782 A1  | 7/2015  | Matsui et al. |                    |
| 2015/0203785 A1  | 7/2015  | Matsui et al. |                    |
| 2015/0322370 A1  | 11/2015 | Matsui et al. |                    |

**FOREIGN PATENT DOCUMENTS**

|    |             |         |
|----|-------------|---------|
| JP | 8-176576    | 7/1996  |
| JP | 2009-506179 | 2/2009  |
| JP | 2012-197399 | 10/2012 |
| JP | 2013-104032 | 5/2013  |
| WO | 2014/017556 | 1/2014  |

**OTHER PUBLICATIONS**

International Search Report dated Oct. 27, 2015 in International (PCT) Application No. PCT/JP2015/076181.

Nakata, "Viscosity index improver for high performance engine oil", Sanyo Chemical News, Sanyo Chemical Industries Ltd., No. 476, 2013, 4 pages, with partial English translation.

\* cited by examiner

*Primary Examiner* — Prem C Singh

*Assistant Examiner* — Francis C Campanell

(74) *Attorney, Agent, or Firm* — Wenderoth, Lind & Ponack, L.L.P.

(57)

**ABSTRACT**

A viscosity index improver comprising a polymer which has a high viscosity index and good shear stability and which exhibits sufficient solubility in a lubricating base oil, a process for producing the same, and a lubricating oil composition containing the viscosity index improver are provided, wherein the viscosity index improver comprising a polymer satisfying the following (1) to (4): (1) weight-average molecular weight (Mw) of 200,000 or more and 600,000 or less; (2) number-average molecular weight (Mn) of 90,000 or more; (3) molecular weight distribution (Mw/Mn) of 4.0 or less; and (4) branching degree of 1.0 or more.

**7 Claims, No Drawings**

**VISCOSITY INDEX IMPROVER, METHOD  
FOR PRODUCING THE SAME AND  
LUBRICATING OIL COMPOSITION**

**TECHNICAL FIELD**

The present invention relates to a viscosity index improver having a specific structure, a method for producing the same, and a lubricating oil composition containing the same. In particular, it relates to a viscosity index improver having a high viscosity index and good shear stability and exhibiting sufficient solubility for a lubricating oil, and a process for producing the same.

**BACKGROUND ART**

In recent years, lubricating oils for internal combustion engines are strongly required to improve fuel economy characteristics, and as one means, reduction of friction loss due to lowering viscosity of a lubricating oil is cited. However, merely lowering the viscosity causes problems such as leakage and burning, so it is effective to add a viscosity index improver having the effect of keeping the viscosity low at low temperature while ensuring high viscosity at high temperature.

As the viscosity index improver, a viscosity index improver containing a polymer is known, and there are various kinds of them. Among them, a viscosity index improver comprising an alkyl (meth)acrylate polymer shows a high viscosity index improving effect. Meanwhile, the viscosity index improver comprising an alkyl (meth)acrylate polymer has a problem that shear stability is poor so that fuel saving characteristics are deteriorated for a long-term use (that is a poor long-life property).

As a means for improving the shear stability, for example, decrease of molecular weight of the polymer contained in the viscosity index improver is cited. In general, the lower the molecular weight, the less susceptible to shear and the smaller the degree of the molecular weight decreasing; and therefore, it is possible to suppress the viscosity lowering after shearing by using a low molecular weight viscosity index improver (refer to Patent Literature 1 and Non-Patent Literature 1). In addition, it has been reported that attempts have been made to improve the shear stability with a polymer having a star structure of which divinylbenzene is used as a core part (refer to Patent Literature 2).

**CITATION LIST**

Patent Literature

Patent Literature 1

Japanese Unexamined Patent Application Publication No. 55 2013-104032

Patent Literature 2

Japanese Unexamined Patent Application Publication No. 50 2012-197399

Non-Patent Literature

Non-Patent Literature 1

Nakata, "Viscosity index improver for high performance engine oil", Sanyo Chemical news, Sanyo Chemical Industries Ltd., 2013, No. 476

**SUMMARY OF INVENTION**

**Technical Problem**

5 However, in general, the lower the molecular weight, the lower the viscosity index improving effect tends to be; and therefore, when a low molecular weight viscosity index improver is used, the problem of lowering the viscosity index occurs. Furthermore, in order to adjust the viscosity to 10 a desired degree, it is necessary to increase the amount of the viscosity index improver to be used, that tends to be disadvantageous in cost. Even when a polymer having a star structure of which divinylbenzene is used as a core part is used, there is still room for improvement in compatibility 15 between the viscosity index and the shear stability.

The present invention has been achieved in view of the above circumstances, and an object of the present invention is to provide a viscosity index improver comprising a polymer which has a high viscosity index and good shear 20 stability and which exhibits sufficient solubility in a lubricating base oil, a process for producing the same, and a lubricating oil composition containing the viscosity index improver.

**Solution to Problem**

The viscosity index improver of the present invention which solves the above problems is a viscosity index improver comprising a polymer which satisfies the following 30 (1) to (4):

- (1) weight-average molecular weight (Mw) of 200,000 or more and 600,000 or less;
- (2) number-average molecular weight (Mn) of 90,000 or more;
- (3) molecular weight distribution (Mw/Mn) of 4.0 or less;
- (4) branching degree of 1.0 or more.

By using the polymer satisfying the above (1) to (4), a viscosity index improver which has a high viscosity index and good shear stability and which exhibits sufficient solubility in a lubricating base oil is obtained.

The viscosity index improver of the present invention preferably comprises a polymer obtained by polymerizing a monomer component in the presence of a tri- or higher functional mercaptan and/or a tri- or higher functional initiator.

As the polymer, a polymer obtained by polymerizing a maleimide monomer (a) represented by the following formula (1), that is referred to as a "component (a)", as an essential component of the monomer component is preferable.



In the above formula, R<sup>1</sup> and R<sup>2</sup> independently represent a hydrogen atom or an alkyl group, and X represents a hydrogen atom, a linear, cyclic or branched alkyl group, which optionally has an aromatic ring, or an aryl group.

As the polymer, a polymer obtained by polymerizing an alkyl (meth)acrylate (b) having an aliphatic hydrocarbon

group of 6 to 40 carbon atoms, that is referred to as a "component (b)", and an alkyl (meth)acrylate (c) having an aliphatic hydrocarbon group of 1 to 5 carbon atoms, that is referred to as a "component (c)", in addition to the component (a) as essential components of the monomer component, is preferable.

Viewing from another aspect, it is preferred that the viscosity index improver of the present invention comprises a polymer having a branch unit derived from a tri- or higher functional mercaptan and/or a branch unit derived from a tri- or higher functional initiator. Furthermore, the polymer preferably has a unit represented by the following formula (4). In the following formula (4), R<sup>1</sup>, R<sup>2</sup> and X represent the same meanings as described above.



The polymer preferably has a unit derived from an alkyl (meth)acrylate having an aliphatic hydrocarbon group of 6 to 40 carbon atoms and a unit derived from an alkyl (meth)acrylate having an aliphatic hydrocarbon group of 1 to 5 carbon atoms in addition to the unit represented by the formula (4).

It is preferred that a content of the unit derived from the component (a) or the unit represented by the formula (4) is 5 parts by mass or more and 30 parts by mass or less, relative to 100 parts by mass of the polymer.

It is preferred that a content of the unit derived from the component (b) or the unit derived from an alkyl (meth)acrylate having an aliphatic hydrocarbon group of 6 to 40 carbon atoms is 50 parts by mass or more and less than 95 parts by mass, relative to 100 parts by mass of the polymer.

The present invention further provides a lubricating oil composition comprising the above-described viscosity index improver.

The present invention further provides a method for producing a viscosity index improver. The method for producing a viscosity index improver of the present invention comprises the step of polymerizing a monomer component in the presence of a tri- or higher functional mercaptan and/or a tri- or higher functional initiator. As the monomer component, it is preferable that a maleimide monomer (a) represented by the above formula (1) is used as an essential component of the monomer component, and more preferable that an alkyl (meth)acrylate (b) having an aliphatic hydrocarbon group of 6 to 40 carbon atoms and an alkyl (meth)acrylate (c) having an aliphatic hydrocarbon group of 1 to 5 carbon atoms are further used.

#### Advantageous Effects of Invention

By using the viscosity index improver of the present invention, shear stability and heat resistance can be improved as compared with a conventional lubricating oil composition. In addition, the viscosity index improver of the present invention facilitates ensuring sufficient solubility in a base oil though it has a high molecular weight, so that it gives a lubricating oil composition having a high viscosity index.

#### DESCRIPTION OF EMBODIMENTS

The present invention will be hereinafter described in detail. In the following description, the term "part" means "part by mass" and the term "%" means "mass %" unless otherwise noted. In addition, the term "A to B" indicating the range means that it is A or more and B or less.

##### [1. Viscosity Index Improver]

A viscosity index improver of the present invention 10 comprises a specific polymer. The polymer used for the viscosity index improver of the present invention can be obtained by radically polymerizing a monomer component that includes a polymerizable monomer having various functional groups in the presence of a tri- or higher functional mercaptan and/or a tri- or higher functional initiator. The polymer according to the present invention can be used 15 for a viscosity index improver.

Examples of the tri- or higher functional mercaptan include polyester compounds formed from a compound 20 having three or more hydroxyl groups and a carboxyl group-containing mercaptan such as trimethylopropane trimercaptoacetate, trimethylopropane tri(3-mercaptopropionate), pentaerythritol tetrakis(mercaptopropionate), pentaerythritol tetrakis(3-mercaptopropionate), 25 dipentaerythritol hexakis(mercaptopropionate) and dipentaerythritol hexakis(3-mercaptopropionate), triazine multifunctional thiols, compounds having three or more mercapto groups per molecule obtained by adding hydrogen sulfide to a plurality of epoxy groups of a multifunctional epoxy 30 compound, compounds having three or more mercapto groups per molecule obtained by esterifying a plurality of carboxyl groups of a multifunctional carboxylic acid and a mercaptoethanol, and the like. Regarding the tri- or higher functional mercaptan, one or more kind of that may be used 35 alone or in combination thereof (for example, by mixing).

The used amount (total amount of addition) of the tri- or higher functional mercaptan may be appropriately determined according to a kind and an amount of a monomer to be used, polymerization conditions such as polymerization 40 temperature and polymerization concentration, molecular weight of the target polymer and others, and is not particularly limited. From a viewpoint of obtaining the viscosity index improver containing a polymer having high base oil solubility and weight-average molecular weight of 100,000 or more, the used amount of the tri- or higher functional mercaptan is preferably 0.01 parts by mass or more, more preferably 0.05 parts by mass or more, and is preferably 5 parts by mass or less, more preferably 3 parts by mass or less, even more preferably 2 parts by mass or less, relative to 45 100 parts by mass of the monomer component. Within this range, molecular weight distribution thereof becomes narrow and the shear stability can be improved.

Examples of the tri- or higher functional initiator include, 50 for example, organic peroxides having three or more functional groups such as 2,2-bis(4,4-t-butylperoxycyclohexyl)propane, tris(t-butylperoxy)triazine, and 3,3',4,4'-tetra(t-butylperoxycarbonyl)benzophenone; however, it is not particularly limited.

The used amount (total amount of addition) of the tri- or higher functional initiator may be appropriately determined 55 according to a purpose and an application, and is not particularly limited. From a viewpoint of obtaining the viscosity index improver containing a polymer having high base oil solubility and weight-average molecular weight of 100,000 or more while considering the balance between polymerizability, adverse effects of decomposed substances and economic efficiency, the used amount of the tri- 60 or

higher functional initiator is preferably 0.01 parts by mass or more, more preferably 0.02 parts by mass or more, even more preferably 0.05 parts by mass or more, and is preferably 10 parts by mass or less, more preferably 5 parts by mass or less, even more preferably 2 parts by mass or less, relative to 100 parts by mass of the monomer component.

A polymer obtained by radical polymerization of a monomer component in the presence of the tri- or higher functional mercaptan and/or the tri- or higher functional initiator has a structure in which polymer chains are branched from the center. That is, the polymer contained in the viscosity index improver of the present invention has a branch unit derived from the tri- or higher functional mercaptan and/or a branch unit derived from the tri- or higher functional initiator. When the polymer contained in the viscosity index improver has such a structure, it is possible to improve shear stability of the viscosity index improver containing the polymer without significantly impairing solubility in a base oil.

In the case where the polymer contained in the viscosity index improver has a branch unit derived from the tri- or higher functional mercaptan, the polymer preferably has a branch unit represented by the following formula (7) (that is a chain transfer agent residue). In the following formula (7),  $L_T$  represents a  $m$ -valent organic residue, and  $m$  represents a number of 0 or more. The  $m$  is preferably 0 to 5.



(7)

In the case where the polymer contained in the viscosity index improver has a branch unit derived from the tri- or higher functional initiator, the polymer preferably has a branch unit derived from a peroxide having three or more functional groups, and specifically, preferably has a branch unit represented by the following formula (8). In the following formula (8),  $L_S$  represents a  $n$ -valent organic residue (an initiator residue), and  $n$  represents a number of 0 or more. The  $n$  is preferably 0 to 5.



(8)

The polymer contained in the viscosity index improver may have either one of the branch unit derived from the tri- or higher functional mercaptan and the branch unit derived from the tri- or higher functional initiator, or may have both of them. Regarding the branch unit derived from the tri- or higher functional mercaptan, only one kind of that may be contained or two or more kinds of that may be contained. Also, regarding the branch unit derived from the tri- or higher functional initiator, only one kind of that may be contained or two or more kinds of that may be contained.

The content of the branch unit derived from the tri- or higher functional mercaptan in the polymer is preferably 0.01 parts by mass or more, more preferably 0.05 parts by mass or more, and is preferably 5 parts by mass or less, more preferably 3 parts by mass or less, even more preferably 2 parts by mass or less, relative to 100 parts by mass of the polymer. Within this range, the molecular weight distribution of the polymer becomes narrow and the shear stability can be improved. The content of the branch unit derived from the tri- or higher functional mercaptan is determined by dividing the used amount of the tri- or higher functional mercaptan by the mass of polymer.

The content of the branch unit derived from the tri- or higher functional initiator in the polymer is preferably 0.01 parts by mass or more, more preferably 0.02 parts by mass or more, even more preferably 0.05 parts by mass or more, and is preferably 10 parts by mass or less, more preferably 5 parts by mass or less, even more preferably 2 parts by mass or less, relative to 100 parts by mass of the polymer, from a viewpoint of obtaining the viscosity index improver containing the polymer having high base oil solubility and a weight-average molecular weight of 100,000 or more in the polymer. The content of the branch unit derived from the tri- or higher functional initiator is determined by dividing the used amount of the tri- or higher functional initiator by the mass of polymer.

The polymer contained in the viscosity index improver of the present invention preferably has a ring structure in the main chain, and the ring structure of the main chain is preferably a succinimide ring structure. Therefore, it is preferred that the polymer contained in the viscosity index improver of the present invention is obtained by polymerizing a maleimide monomer (a) represented by the following formula (1) (that is hereinafter referred to as a "component (a)") as an essential component of the monomer component.



(1)

In the above formula (1),  $R^1$  and  $R^2$  independently represent a hydrogen atom or an alkyl group, and  $X$  represents a hydrogen atom, a linear, cyclic or branched alkyl group, which includes an alkyl group having an aromatic ring, or an aryl group. In the case where the  $X$  is an alkyl group, the alkyl group may be linear, cyclic or branched, and any substituent may be bonded to the alkyl group. The substituent may have an aromatic ring (for example, a phenyl group). In the case where the  $X$  is an aryl group, any substituent may be bonded to the aryl group.

In the case where the  $X$  is an alkyl group, it is preferred that the alkyl group has a cyclic structure, and as such alkyl group, an alkyl group having an aromatic ring (that is, an aralkyl group) such as a benzyl group and a cycloalkyl group such as a cyclohexyl group are preferable. As the aryl group, a phenyl group, a naphthyl group and an aryl group in which hydrogen of an aromatic ring is substituted are preferable.

Specific examples of the monomer component (a) include maleimide; a maleimide in which a linear or branched alkyl group of 1 to 20 carbon atoms is bonded to a nitrogen atom such as N-methylmaleimide, N-ethylmaleimide, N-isopro-

pylmaleimide, N-butylnaleimide, N-isobutylmaleimide, N-tert-butylmaleimide, N-cyclohexylmaleimide, N-laurylmaleimide and N-stearylmaleimide; a maleimide in which a cyclic alkyl group of 5 to 10 carbon atoms is bonded to a nitrogen atom such as N-cyclohexylmaleimide; a maleimide in which an aryl group or aralkyl group of 6 to 12 carbon atoms bonded to a nitrogen atom such as N-phenylmaleimide, N-benzylmaleimide, N-chlorophenylmaleimide, N-methylphenylmaleimide, N-naphthylmaleimide, N-hydroxylphenylmaleimide, N-methoxyphenylmaleimide, N-carboxyphenylmaleimide, N-nitrophenylmaleimide and N-tribromophenylmaleimide; a maleimide in which a hydroxyl alkyl group is bonded to a nitrogen atom such as N-hydroxylethylmaleimide; and others. Among them, N-phenylmaleimide, N-cyclohexylmaleimide, N-isopropylmaleimide, N-benzylmaleimide, N-laurylmaleimide and N-stearylmaleimide are preferable in view of availability, economic efficiency and high solubility in a base oil. The above monomer component (a) may be used alone or in combination of two or more kinds.

By polymerizing a monomer component including the component (a), a polymer having a unit represented by the following formula (4), that is, a polymer having a succinimide ring structure in the main chain, is obtained. Therefore, the polymer contained in the viscosity index improver of the present invention preferably has a unit represented by the following formula (4). In the following formula (4), R<sup>1</sup>, R<sup>2</sup> and X represent the same meanings as described above.



The content of the monomer component (a) is preferably 0.5 parts by mass or more, more preferably 2 parts by mass or more, even more preferably 5 parts by mass or more, and is preferably 35 parts by mass or less, more preferably 30 parts by mass or less, relative to 100 parts by mass of the total monomer components. The content of the unit derived from the monomer component (a) (that is, the unit represented by the above formula (4)) in the polymer is preferably 0.5 parts by mass or more, more preferably 2 parts by mass or more, even more preferably 5 parts by mass or more, and is preferably 35 parts by mass or less, more preferably 30 parts by mass or less, relative to 100 parts by mass of the polymer. The viscosity index improver containing the polymer obtained by using the monomer component (a) in the above range or the polymer having the unit derived from the monomer component (a) in the above range enables to enhance the shear stability while maintaining solubility in a base oil. Furthermore, it is expected to improve detergency and dispersibility of sludge and the like, and to suppress abrasion of a metal surface.

The polymer contained in the viscosity index improver of the present invention is preferably a (meth)acrylate polymer having a cyclic structure in the main chain, and more preferably, a polymer obtained by polymerizing an alkyl (meth)acrylate (b) having an aliphatic hydrocarbon group of 6 to 40 carbon atoms (that is hereinafter referred to as a "component (b)") and an alkyl (meth)acrylate (c) having an

aliphatic hydrocarbon group of 1 to 5 carbon atoms (that is hereinafter referred to as a "component (c)") in addition to the component (a) as essential components of the monomer component.

As the monomer component (b), a (meth)acrylate represented by the following formula (2) is preferable. In the following formula (2), R<sup>3</sup> represents a hydrogen atom or a methyl group, and R<sup>4</sup> represents an alkyl group of 6 to 40 carbon atoms (preferably an alkyl group of 6 to 24 carbon atoms, and more preferably an alkyl group of 12 to 24 carbon atoms). The alkyl group of R<sup>4</sup> may be linear, cyclic or branched, and may have a substituent.



The monomer component (b) may be a monomer in which R<sup>3</sup> and R<sup>4</sup> are respectively single kinds, or may be a mixture of two or more monomers in which R<sup>3</sup> and/or R<sup>4</sup> are different from each other. In view of reactivity, R<sup>3</sup> is preferably a hydrogen atom or a methyl group.

Specific examples of the monomer component (b) include n-hexyl (meth)acrylate, 2-ethylhexyl (meth)acrylate, n-octyl (meth)acrylate, nonyl (meth)acrylate, decyl (meth)acrylate, undecyl (meth)acrylate, dodecyl (meth)acrylate, tridecyl (meth)acrylate, tetradecyl (meth)acrylate, pentadecyl (meth)acrylate, hexadecyl (meth)acrylate, heptadecyl (meth)acrylate, stearyl (meth)acrylate, nonadecyl (meth)acrylate, eicosyl (meth)acrylate, behenyl (meth)acrylate, tetracosyl (meth)acrylate, 2-decytetradecyl (meth)acrylate, cyclohexyl (meth)acrylate, menthyl (meth)acrylate, isobornyl (meth)acrylate, dicyclopentanyl (meth)acrylate, adamantyl (meth)acrylate, and others. Among them, in view of availability, economic efficiency and high solubility in a base oil, 2-ethylhexyl (meth)acrylate, dodecyl (meth)acrylate, stearyl (meth)acrylate, eicosyl (meth)acrylate, behenyl (meth)acrylate, tetracosyl (meth)acrylate, 2-decytetradecyl (meth)acrylate and cyclohexyl (meth)acrylate are preferable. The above monomer component (b) may be used alone or in combination of two or more kinds.

By polymerizing a monomer component including the component (b), a unit derived from an alkyl (meth)acrylate having an aliphatic hydrocarbon group of 6 to 40 carbon atoms is introduced into the polymer. Therefore, the polymer contained in the viscosity index improver of the present invention preferably has a unit derived from an alkyl (meth)acrylate having an aliphatic hydrocarbon group of 6 to 40 carbon atoms, in addition to the unit represented by the above formula (4), and more preferably has a unit represented by the following formula (5). In the following formula (5), R<sup>3</sup> and R<sup>4</sup> represent the same meanings as described above.



The content of the monomer component (b) is preferably 50 parts by mass or more, more preferably 55 parts by mass or more, and is preferably less than 95 parts by mass, more preferably 93 parts by mass or less, even more preferably 90 parts by mass or less, relative to 100 parts by mass of the total monomer components. The content of the unit derived from the monomer component (b) (that is, the unit derived from an alkyl (meth)acrylate having an aliphatic hydrocarbon group of 6 to 40 carbon atoms) in the polymer is preferably 50 parts by mass or more, more preferably 55 parts by mass or more, and is preferably less than 95 parts by mass, more preferably 93 parts by mass or less, even more preferably 90 parts by mass or less, relative to 100 parts by mass of the polymer. The viscosity index improver containing the polymer obtained by using the monomer component (b) in the above range or the polymer having the unit derived from the monomer component (b) in the above range comes to have high solubility in base oils of various compositions.

As the monomer component (c), a (meth)acrylate represented by the following formula (3) is preferable. In the following formula (3), R<sup>5</sup> represents a hydrogen atom or a methyl group, and R<sup>6</sup> represents an aliphatic hydrocarbon group of 1 to 5 carbon atoms (preferably an alkyl group of 1 to 5 carbon atoms). The aliphatic hydrocarbon group of R<sup>6</sup> may be linear, cyclic or branched, and may have a substituent.



The monomer component (c) may be a monomer in which R<sup>5</sup> and R<sup>6</sup> are respectively a single kinds, or may be a mixture of two or more monomers in which R<sup>5</sup> and/or R<sup>6</sup> are different from each other. In view of reactivity, R<sup>5</sup> is preferably a hydrogen atom or a methyl group. In addition, in view of improving a viscosity index, it is preferable that the aliphatic hydrocarbon group of R<sup>6</sup> is linear or branched.

Specific examples of the monomer component (c) include, for example, methyl (meth)acrylate, ethyl (meth)acrylate, n-propyl (meth)acrylate, iso-propyl (meth)acrylate, n-butyl (meth)acrylate, iso-butyl (meth)acrylate, t-butyl (meth)acrylate, n-amyl (meth)acrylate, iso-amyl (meth)acrylate, t-amyl (meth)acrylate, neopentyl (meth)acrylate, and others. In particular, it is preferable that at least methyl (meth)acrylate is included as the monomer component (c). When the monomer component (c) includes methyl (meth)acrylate, the viscosity index improver which exhibits a high viscosity index improvement effect and has high heat resistance and shear stability is obtained. The above monomer component (c) may be used alone or in combination of two or more kinds.

By polymerizing a monomer component including the component (c), a unit derived from an alkyl (meth)acrylate having an aliphatic hydrocarbon group of 1 to 5 carbon atoms is introduced into the polymer. Therefore, the polymer contained in the viscosity index improver of the present invention preferably has a unit derived from an alkyl (meth)acrylate having all aliphatic hydrocarbon group of 1 to 5 carbon atoms, in addition to the unit represented by the above formula (4), and more preferably has a unit repre-

sented by the following formula (6). In the following formula (6), R<sup>5</sup> and R<sup>6</sup> represent the same meanings as described above. More preferably, the polymer contained in the viscosity index improver of the present invention has a unit derived from an alkyl (meth)acrylate having an aliphatic hydrocarbon group of 6 to 40 carbon atoms and a unit derived from all alkyl (meth)acrylate having an aliphatic hydrocarbon group of 1 to 5 carbon atoms, in addition to the unit represented by the above formula (4).



The content of the monomer component (c) is preferably 2 parts by mass or more, more preferably 5 parts by mass or more, and is preferably 40 parts by mass or less, more preferably 35 parts by mass or less, even more preferably 30 parts by mass or less, relative to 100 parts by mass of the total monomer components. The content of the unit derived from the monomer component (c) (that is, the unit derived from an alkyl (meth)acrylate having an aliphatic hydrocarbon group of 1 to 5 carbon atoms) in the polymer is preferably 2 parts by mass or more, more preferably 5 parts by mass or more, and is preferably 40 parts by mass or less, more preferably 35 parts by mass or less, even more preferably 30 parts by mass or less, relative to 100 parts by mass of the polymer. When the content of the monomer component (c) or the content of the unit derived from the monomer component (c) is in the above range, copolymerizability with other components is good, polymerization velocity is enhanced, a polymerization rate is high, and productivity is good. In addition, the shear stability and the base oil solubility of the viscosity index improver obtained by copolymerization are further improved.

The monomer component for synthesizing the polymer of the present invention may contain a radically polymerizable monomer other than the components (a), (b) and (c) (that is hereinafter referred to as a "component (d)"). The radically polymerizable monomer of the component (d) is classified into a monofunctional monomer having one radically polymerizable group in the molecule and a multifunctional monomer having two or more radically polymerizable groups in the molecule.

Examples of the monofunctional monomer include (meth)acrylates other than the components (b) and (c), unsaturated mono- or dicarboxylate esters, unsaturated carboxylic acids, vinylaromatic compounds, vinyl esters, vinyl ethers, olefins, vinyl cyanide, N-vinyl compounds, (meth)acrylamide and others. These monofunctional monomers may be used alone, or two or more kinds of them may be used in combination.

Examples of the (meth)acrylate other than the components (b) and (c) include, for example, benzyl (meth)acrylate, phenyl (meth)acrylate, 2-hydroxyethyl (meth)acrylate, 2-hydroxybutyl (meth)acrylate, 2-methoxyethyl (meth)acrylate, tetrahydrofurfuryl (meth)acrylate, N,N-dimethylaminoethyl (meth)acrylate, morpholinoalkylene (meth)acrylate, methyl  $\alpha$ -hydroxymethylacrylate, polyethyleneglycol mono(meth)acrylate and others.

Examples of the unsaturated mono- or dicarboxylate ester include, for example, butyl crotonate, octyl crotonate, dibutyl maleate, dilauryl maleate, dioctyl fumarate, distearyl fumarate and others.

## 11

Examples of the unsaturated carboxylic acid include, for example, (meth)acrylic acid, maleic acid, fumaric acid, maleic anhydride and others.

Examples of the vinyl aromatic compound include, for example, styrene monomers such as styrene,  $\alpha$ -methyl styrene, vinyl toluene and methoxystyrene, 2-vinyl pyridine, 4-vinyl pyridine and others.

Examples of the vinyl ester include, for example, vinyl acetate, vinyl propionate, vinyl octylate and others.

Examples of the vinyl ether include, for example, methyl vinyl ether, butyl vinyl ether, octyl vinyl ether, dodecyl vinyl ether and others.

Examples of the olefin include, for example, ethylene, propylene, 1-butene, isobutene, 1-tetradecene, 1-octadecene, diisobutene and others.

Examples of the vinyl cyanide include, for example, acrylonitrile, methacrylonitrile and others.

Examples of the N-vinyl compound include, for example, N-vinylpyrrolidone, N-vinylcaprolactam, N-vinylimidazole, N-vinylmorpholine, N-vinylacetamide and others.

Examples of the (meth)acrylamide include, for example, N,N-dimethyl (meth)acrylamide, N,N-diethyl (meth)acrylamide, N,N-dibutyl (meth)acrylamide, N-methylol (meth)acrylamide, acryloyl morpholine and others.

Among these monofunctional monomers, 2-hydroxyethyl (meth)acrylate, N,N-dimethylaminoethyl (meth)acrylate, methyl  $\alpha$ -hydroxymethylacrylate, N-vinylpyrrolidone, N,N-dimethyl (meth)acrylamide and acryloyl morpholine are preferable.

The content of the monofunctional monomer of the monomer component (d) is preferably 0 parts by mass or more and 30 parts by mass or less, more preferably 25 parts by mass or less, and even more preferably 20 parts by mass or less, relative to 100 parts by mass of the total monomer components. The content of the unit derived from the monofunctional monomer of the component (d) in the polymer is preferably 0 parts by mass or more and 30 parts by mass or less, more preferably 25 parts by mass or less, and even more preferably 20 parts by mass or less, relative to 100 parts by mass of the polymer.

However, in the case of using the styrene monomer, the content of the styrene monomer is preferably 2 parts by mass or less, relative to 100 parts by mass of the total monomer components. The content of the unit derived from the styrene monomer in the polymer is preferably 2 parts by mass or less, relative to 100 parts by mass of the polymer. When the content of the unit derived from the styrene monomer exceeds 2 parts by mass, solubility in a base oil and a viscosity index of the viscosity index improver containing the polymer tend to be lowered.

In the case where olefin is used as the monomer, the content of olefin is preferably 5 parts by mass or less and more preferably 3 parts by mass or less, relative to 100 parts by mass of the total monomer components. The content of unit derived from olefin in the polymer is preferably 5 parts by mass or less and more preferably 3 parts by mass or less, relative to 100 parts by mass of the polymer. When the content of unit derived from olefin exceeds 5 parts by mass, a viscosity index of the viscosity index improver containing the polymer tends to be lowered.

Examples of the multifunctional monomer of the monomer component (d) include multifunctional (meth)acrylic compounds such as a multifunctional (meth)acrylate, a vinyl ether group-containing (meth)acrylate, an allyl group-containing (meth)acrylate, a multifunctional (meth)acryloyl group-containing isocyanurate and a multifunctional urethane (meth)acrylate, multifunctional maleimide com-

## 12

pounds, multifunctional vinyl ethers, multifunctional allyl compounds, multifunctional aromatic vinyl compounds and others. These multifunctional monomers may be used alone or in combination of two or more.

Examples of the multifunctional (meth)acrylate (that is a multifunctional (meth)acrylate ester) include, for example, ethyleneglycol di(meth)acrylate, diethyleneglycol di(meth)acrylate, polyethyleneglycol di(meth)acrylate, hexanediol di(meth)acrylate, bisphenol-A alkylene oxide di(meth)acrylate, trimethylolpropane tri(meth)acrylate, 2,2'-(oxybis(methylene)] bisacrylic acid, dialkyl-2,2'-(oxybis(methylene)] bis-2-propenoate and others.

Examples of the vinyl ether group-containing (meth)acrylate (that is a vinyl ether group-containing (meth)acrylate ester) include, for example, 2-vinylxyethyl (meth)acrylate, 4-vinylxybutyl (meth)acrylate, 2-(vinylxyethoxy)ethyl (meth)acrylate and others.

Examples of the allyl group-containing (meth)acrylate (that is an allyl group-containing (meth)acrylate ester) include, for example, allyl (meth)acrylate, methyl  $\alpha$ -allyloxyethylacrylate, stearyl  $\alpha$ -allyloxyethylacrylate, 2-decytetradecyl  $\alpha$ -allyloxyethylacrylate and others.

Examples of the multifunctional (meth)acryloyl group-containing isocyanurate include, for example, tri(acryloyloxyethyl) isocyanurate, tri(methacryloyloxyethyl) isocyanurate and others.

Examples of the multifunctional urethane (meth)acrylate (that is a multifunctional urethane (meth)acrylate ester) include, for example, a multifunctional urethane (meth)acrylate obtained by the reaction of a multifunctional isocyanate such as tolylene diisocyanate, isophorone diisocyanate and xylylene diisocyanate, with a hydroxyl group-containing (meth)acrylate ester such as 2-hydroxyethyl (meth)acrylate and 2-hydroxypropyl (meth)acrylate, and others.

Examples of the multifunctional maleimide compound include, for example, 4,4'-diphenylmethane bismaleimide, m-phenylene bismaleimide, bisphenol-A diphenyl ether bismaleimide, 1,6-bismaleimide-(2,2,4-trimethyl)hexane and others.

Examples of the multifunctional vinyl ether include, for example, ethyleneglycol divinyl ether, diethyleneglycol divinyl ether, polyethyleneglycol divinyl ether, hexanediol divinyl ether, bisphenol-A alkylene oxide divinyl ether, trimethylolpropane trivinyl ether and others.

Examples of the multifunctional allyl compound include, for example, multifunctional allyl ethers such as ethyleneglycol diallyl ether, diethyleneglycol diallyl ether, polyethyleneglycol diallyl ether, hexanediol diallyl ether, bisphenol-A alkylene oxide diallyl ether, trimethylolpropane triallyl ether and ditrimethylolpropane tetraallyl ether; multifunctional allyl group-containing isocyanurates such as triallyl isocyanurate; multifunctional allyl esters such as diallyl phthalate and diallyl diphenate; bisallylnadiimide compounds; bisallylnadiimide compounds and others.

Examples of the multifunctional aromatic vinyl compound include, for example, divinylbenzene and others.

The content of the multifunctional monomer of the monomer component (d) is preferably 0 parts by mass or more and 5 parts by mass or less, more preferably 3 parts by mass or less, and even more preferably 2 parts by mass or less, relative to 100 parts by mass of the total monomer components. The content of the unit derived from the multifunctional monomer of the component (d) in the polymer is preferably 0 parts by mass or more and 5 parts by mass or less, more preferably 3 parts by mass or less, and even more preferably 2 parts by mass or less, relative to 100 parts by

mass of the polymer. In this case, the shear stability of the viscosity index improver containing the polymer can be improved without significantly impairing the solubility in a base oil, due to adopting a branched structure of the polymer or the like.

However, in the case of a multifunctional monomer that undergoes polymerization while cycling, such as 2,2'-[oxybis(methylene)] bisacrylic acid, dialkyl-2,2'-[oxybis(methylene)] bis-2-propenoate, methyl  $\alpha$ -allyloxymethylacrylate, stearyl  $\alpha$ -allyloxymethylacrylate and 2-decytetradecyl  $\alpha$ -allyloxymethylacrylate, the content of the unit derived from such multifunctional monomer in the polymer is preferably 0 parts by mass or more and 30 parts by mass or less, more preferably 25 parts by mass or less, and even more preferably 20 parts by mass or less, relative to 100 parts by mass of the polymer. The same is also applied to the content of the multifunctional monomer relative to 100 parts by mass of the total monomer components. In this case, due to the effect of introducing a ring structure into the main chain, heat resistance of the viscosity index improver containing the polymer can be improved and the shear stability is improved.

When the unit derived from the multifunctional monomer exceeds the above range, gelation may proceed during polymerization or solubility of the viscosity index improver containing the polymer in a base oil may be deteriorated.

The viscosity index improver of the present invention can be obtained by a production method comprising the step of polymerizing a monomer component in the presence of tri- or higher functional mercaptan and/or tri- or higher functional initiator (that is a polymerization step). A polymerization method of the monomer component in the polymerization step may be, for example, bulk polymerization, solution polymerization, suspension polymerization, emulsion polymerization or the like, and is not particularly limited. In the case of using a dispersion medium, an emulsifying agent, a dispersing agent or the like, there is no particular limitation on them and known ones can be used.

Preferable conditions such as the kind and amount of the tri- or higher functional mercaptan and/or the tri- or higher functional initiator used in the polymerization step are as described above. At the time of polymerization, the tri- or higher functional mercaptan and/or the tri- or higher functional initiator may be added all at once or dividedly. A bi- or less functional mercaptan or a bi- or less functional initiator may be used in combination.

In the polymerization step, it is preferable to essentially use the above-mentioned monomer (a) as the monomer component. Moreover, it is more preferable to further use the above-mentioned monomer component (b) and the monomer component (c) in addition to the monomer component (a). As the monomer component, the above-mentioned monomer component (d) may be used in combination. Preferable conditions such as the type and used amount of each of these monomer components are as described above.

A solvent used for the polymerization is not particularly limited as long as it is inactive to the polymerization reaction, and can be appropriately selected according to the polymerization mechanism, the kind and amount of the monomer used, the kind and amount of the polymerization initiator or a polymerization catalyst and the like. From a viewpoint of ensuring solubility of the polymer and easy solvent replacement to a base oil after polymerization, toluene, xylene, hexane, cyclohexane, methyl ethyl ketone or tetrahydrofuran is preferably used as the solvent for polymerization. Or, a lubricating base oil described below

can also be suitably used as the solvent. In this case, solvent replacement after polymerization is unnecessary and the process is simplified, that is more preferable. These solvents may be used alone, or two or more of them may be used in combination. The used amount of the solvent is not particularly limited, and from a viewpoint of obtaining the polymer having weight-average molecular weight of 100,000 or more, it is preferable that the concentration of the total amount of the monomer component, the polymerization initiator and other components is about 40 mass % or more and 100 mass % or less.

In the polymerization step, an acidic substance may be used as an additive in polymerizing the monomer component. By using an acidic substance, the Michael addition reaction between the monomer component (a) and the tri- or higher functional mercaptan can be suppressed, and the unit derived from the monomer component (a) can be efficiently introduced into the polymer. In addition, a polymerization rate of each monomer other than the component (a) may increase.

The acidic substance is not particularly limited, as long as it is able to adjust the pH in the range of 2.0 to 6.5 (preferably pH 3.0 to 5.5) when a certain amount of that is added to water of the same mass as all the components such as the monomers and solvents used for polymerization, and for example, an organophosphorus compound or an organic acid is preferably used. Examples of the organic phosphorus compound include alkyl (aryl) phosphorous acid and monoester thereof, dialkyl (aryl) phosphinic acid, alkyl (aryl) phosphonic acid and monoester thereof, alkylphosphinic acid, di- or monoester of phosphorous acid, di- or monoester of phosphoric acid and others. Examples of the organic acid include acetic anhydride, propionic anhydride, phthalic anhydride and others. These organophosphorus compounds or organic acids may be used alone, or two or more of them may be used in combination. The used amount of the acidic substance may be 0 mass % or more, preferably 5 mass % or less, more preferably 1 mass % or less, and even more preferably 0.5 mass % or less, relative to 100 parts by mass of the total monomer component.

Polymerization temperature in polymerizing the monomer component is not particularly limited, and may be appropriately set according to the polymerization mechanism, the kind and amount of the monomer used, the kind and amount of the polymerization initiator or a polymerization catalyst and the like; however, it is preferably 0° C. or higher, more preferably 25° C. or higher, and is preferably 200° C. or lower, more preferably 150° C. or lower. When the polymerization temperature is lower than 0° C., the polymerization reaction becomes extremely slow, and when it exceeds 200° C., the reaction becomes severe and the control becomes difficult; and thus, it is not preferable either.

The weight-average molecular weight (Mw) of the polymer contained in the improver of the present invention is preferably 100,000 or more, more preferably 200,000 or more, even more preferably 300,000 or more, still even more preferably 360,000 or more, and is preferably 600,000 or less, more preferably 580,000 or less, even more preferably 550,000 or less. When the weight-average molecular weight of the polymer is less than the above lower limit value, the viscosity index of the lubricating oil composition is made low, and it becomes necessary to increase the used amount of the viscosity index improver in order to adjust the viscosity to a desired degree, that is disadvantageous in terms of cost. When the weight-average molecular weight of the polymer is excessively large, solubility of the viscosity

index improver in a base oil tends to be insufficient and the shear stability of the lubricating oil composition tends to decrease.

The number-average molecular weight ( $M_n$ ) of the polymer contained in the viscosity index improver of the present invention is preferably 90,000 or more, more preferably in the range of 90,000 to 300,000 and even more preferably in the range of 90,000 to 200,000.

The molecular weight distribution ( $M_w/M_n$ ) calculated from the  $M_w$  and the  $M_n$  is preferably 4.0 or less, more preferably 3.5 or less and even more preferably 3.0 or less. When the molecular weight distribution exceeds 4.0, solubility of the viscosity index improver in a base oil may become insufficient or the shear stability of the lubricating oil composition may decrease, that is undesirable. Meanwhile, the lower limit of the molecular weight distribution is preferably 1.0; however, in view of easily synthesis of the polymer, the molecular weight distribution ( $M_w/M_n$ ) is preferably 1.5 or more, more preferably 2.0 or more and even more preferably 2.3 or more. In the present invention, the  $M_w$  and the  $M_n$  are values measured by the methods described in Examples of described below.

As a method for controlling the molecular weight, a known method can be employed. For example, it can be controlled by adjusting the amount and kind of the polymerization initiator or a polymerization catalyst, polymerization temperature, the kind and amount of the chain transfer agent, and the like. As a method of controlling the molecular weight distribution, living radical polymerization can also be employed. As a specific method, the RAFT method, the NMP method, the ATRP method and the like are famous. More information is outlined in Aldrich Material Matters, Vol. 5, No. 1, 2010. As an example of use, for example in the case of the RAFT method, 2,2'-azobisisobutyronitrile as a polymerization initiator and cumyl dithiobenzoate as a polymerization catalyst are used in JP-A-2012-197399.

Branching degree of the polymer contained in the viscosity index improver of the present invention is preferably 1.0 or more, more preferably 1.4 or more, and is preferably 10.0 or less, more preferably 6.0 or less, even more preferably 4.0 or less. When the branching degree is less than 1.0, the branched structure of the polymer is not sufficient and improvement of the shear stability is not expected. The branching degree in the present invention corresponds to the average of number of branch points per molecule of the polymer and is a value measured by the method described in Examples below. Logically, for example, the branching degree of a straight chain polymer without branching is 0, the branching degree of a polymer in which three polymer chains extend from only one branch point is 1, the branching degree of a polymer in which four polymer chains extend from that is 2, and the branching degree of a polymer in which five polymer chains extend from that is 3.

The content of the polymer described above in the viscosity index improver is not particularly limited as long as it does not impair the effect of the present invention; however, the viscosity index improver of the present invention preferably contains the above-described polymer as a main component. The content of the polymer in the viscosity index improver is, for example, preferably 50 parts by mass or more, more preferably 80 parts by mass or more and even more preferably 90 parts by mass or more, relative to 100 parts by mass of the viscosity index improver. The viscosity index improver may substantially consist of only the above-described polymer.

The SP value (solubility parameter) of the polymer contained in the viscosity index improver of the present invention

is preferably 9.0 or higher, more preferably 9.1 or higher, even more preferably 9.2 or higher, and is preferably 9.6 or lower, more preferably 9.5 or lower, even more preferably 9.4 or lower. The SP value of a base oil generally has a value of about 8.0 to 8.5, and when the SP value of the polymer is 9.0 or higher, the viscosity index of the lubricating oil composition is easily increased, and when the SP value is 9.6 or lower, solubility of the viscosity index improver in a base oil is easily ensured. The SP value is obtained by a method described in Examples below.

The viscosity index improver of the present invention is able to attain a viscosity index improvement effect and shear stability at a high level. As a specific numerical value of the shear stability, PSSI (Permanent Shear Stability index: ASTM D 6022) or decomposition starting temperature can be used as an indicator.

The PSSI of the viscosity index improver is preferably 40 or less, more preferably 35 or less, even more preferably 30 or less, and particularly preferably 25 or less. The PSSI is preferably 0.1 or more, more preferably 0.5 or more, even more preferably 2 or more, and particularly preferably 5 or more. When the PSSI is less than 0.1, the viscosity index improving effect is small and the cost may be increased. When the PSSI exceeds 40, the shear stability and storage stability may be deteriorated.

The decomposition starting temperature of the viscosity index improver is preferably 290°C. or higher, more preferably 295°C. or higher, even more preferably 300°C. or higher, particularly preferably 310°C. or higher, and is preferably 500°C. or lower, more preferably 450°C. or lower, even more preferably 400°C. or lower, particularly preferably 380°C. or lower. When the decomposition starting temperature of the viscosity index improver is raised, heat resistance is enhanced and the thermal decomposition stability and the shear stability are improved. Meanwhile, when the heat resistance is excessively increased, solubility in the base oil tends to be insufficient and the viscosity index tends to decrease.

The viscosity index improver of the present invention contains the above-described polymer as a main component, and preferably contains 70 mass % or more, more preferably 90 mass % or more, even more preferably 95 mass % or more, particularly preferably 99 mass % or more and 100 mass % or less of the polymer in 100 mass % of the viscosity index improver.

## [2. Composition Containing Viscosity Index Improver and Base Oil]

The present invention also provides a lubricating oil composition containing the viscosity index improver of the present invention. Blending the viscosity index improver of the present invention with a lubricating base oil gives a lubricating oil composition. The lubricating oil composition may be used as a lubricating oil without further diluted with a lubricating base oil or may be diluted with a lubricating base oil to use as a lubricating oil. In the latter case, the lubricating oil composition is used as a stock solution, that may hereinafter be referred to as a "base oil composition".

As the lubricating base oil, a known lubricating base oil can be used without particular limitation, and a mineral base oil and a synthetic base oil are suitably cited. Examples of the mineral base oil include a paraffin-base base oil and a naphthen-base base oil. The mineral base oil include that obtained by subjecting a raw material base oil to solvent refining, hydrocracking or hydroisomerization treatment. Examples of the synthetic base oil include a hydrocarbon-base base oil, an ester-base base oil, an ether-base base oil, a silicone-base base oil and a fluorine-base base oil. As

described above, the lubricating base oil can also be used as the solvent for polymerization for obtaining the polymer contained in the viscosity index improver.

Preferred specific examples of the mineral base oil include base oils obtained by purifying the following base oils (1) to (7) as raw material oils and/or a lubricating oil fraction recovered from this raw material oil using a predetermined purification method and recovering a lubricating oil fraction. Specifically, the following base oils (8) and (9), which are obtained by subjecting a base oil selected from the following (1) to (7) or a lubricating oil fraction recovered from this base oil to a predetermined treatment, are preferable.

- (1) distillate oil (WVGO) obtained by vacuum distillation of an atmospheric distillation residual oil of a paraffin-base crude oil and/or a mixed-base crude oil;
- (2) wax obtained by a dewaxing process of a lubricating oil (slack wax and the like) and/or synthetic wax obtained by a gas to liquid (GTL) process and the like (Fischer Tropsch wax, GTL wax, and the like);
- (3) mixed oil of one or more kinds selected from the base oils (1) to (2) and/or a mild hydrocracking-treated oil of this mixed oil;
- (4) mixed oil of two or more kinds selected from the base oils (1) to (3);
- (5) deasphalted oil (DAO) of any one of the base oils (1) to (4);
- (6) mild hydrocracking-treated oil (MHC) of the base oil (5);
- (7) mixed oil of two or more kinds selected from the base oils (1) to (6);
- (8) hydrocracked mineral oil obtained by hydrocracking the base oil selected from the base oils (1) to (7) or a lubricating oil fraction recovered from this base oil, subjecting its product or a lubricating oil fraction recovered from its product by distillation or the like to a dewaxing treatment such as solvent dewaxing or catalytic dewaxing, and further optionally distilling after the dewaxing treatment;
- (9) hydroisomerized mineral oil obtained by hydroisomerizing the base oil selected from the base oils (1) to (7) or a lubricating oil fraction recovered from this base oil, subjecting its product or a lubricating oil fraction recovered from its product by distillation or the like to a dewaxing treatment such as solvent dewaxing or catalytic dewaxing, and further optionally distilling after the dewaxing treatment.

Specific examples of the synthetic base oil include poly- $\alpha$ -olefins or hydrides thereof, isobutene oligomers or hydrides thereof, isoparaffins, alkylbenzenes, alkylnaphthalenes, diesters such as ditridecylglutarate, di-2-ethylhexyl adipate, diisodecyl adipate, ditridecyl adipate and di-2-ethylhexyl sebacate, polyol esters such as trimethylolpropane caprylate, trimethylolpropane pelargonate, pentaerythritol 2-ethylhexanoate and pentaerythritol pelargonate, polyoxyalkylene glycols, dialkyl diphenyl ethers, polyphenyl ethers and others; and among them, poly- $\alpha$ -olefins are preferable. Typical examples of the poly- $\alpha$ -olefin include oligomers or co-oligomers of  $\alpha$ -olefin having 2 to 32 carbon atoms, preferably 6 to 16 carbon atoms, such as 1-octene oligomer, decene oligomer and ethylene-propylene co-oligomer, and hydrides thereof. Kinematic viscosity of the synthetic base oil at 100° C. is preferably 1 to 20 mm<sup>2</sup>/s.

As the lubricating base oil to be blended in the lubricating oil composition, the base oil (8) or (9), that is obtained by subjecting the base oil selected from the base oils (1) to (7) or a lubricating oil fraction recovered from this base oil to the above-described treatment, is particularly preferred. It is

also preferable to use base oils belonging to Group III based on the classification by the American Petroleum Institute (API). As the lubricating base oil to be blended in the lubricating oil composition, the synthetic base oil described above may be used.

In the lubricating oil composition of the present invention, the above-described lubricating base oil may be used singly or in combination with one or more of other base oils. In the case of using the lubricating base oil and another base oil in combination to prepare a mixed base oil, the mixed base oil preferably contains at least the lubricating base oil (8) or (9). The ratio of the lubricating base oil (8) or (9) in the mixed base oil is preferably 30 mass % or more, more preferably 50 mass % or more and even more preferably 70 mass % or more.

The viscosity index of the lubricating base oil is preferably 100 or higher, more preferably 120 or higher, and is preferably 160 or lower. When the viscosity index is less than the above lower limit value, friction coefficient tends to increase, thereby decreasing anti-wear property, as well as viscosity-temperature characteristic, the heat/oxidation stability and volatilization prevention property deteriorate. When the viscosity index exceeds the above upper limit value, low-temperature viscosity characteristic tends to deteriorate. Here, the viscosity index referred to in the present invention means a viscosity index measured in accordance with JIS K 2283.

The viscosity index of the lubricating oil composition is preferably 200 or higher, more preferably 230 or higher, and is preferably 400 or lower, more preferably 300 or lower. When the viscosity index is within this range, it is excellent in fuel economy, heat/oxidation stability and storage stability.

The content of the viscosity index improver of the present invention in the lubricating oil composition is not particularly limited, and for example, it is preferably 0.01 mass % or more, more preferably 0.1 mass % or more, even more preferably 0.5 mass % or more, and is preferably 70 mass % or less, more preferably 60 mass % or less, even more preferably less than 50 mass %, based on the total amount of the lubricating oil composition. In the case where the lubricating oil composition is used as a lubricating oil without further diluted with a lubricating base oil, the content of the viscosity index improver of the present invention in the lubricating oil composition is preferably 0.01 mass % or more, more preferably 0.1 mass % or more, even more preferably 0.5 mass % or more, and is preferably 20 mass % or less, more preferably 15 mass % or less, even more preferably 10 mass % or less, based on the total amount of the lubricating oil composition. In the case where the lubricating oil composition of the present invention is used as the base oil composition, the content of the viscosity index improver of the present invention in the base oil composition is preferably, for example, 5 mass % or more, more preferably 10 mass % or more, even more preferably 20 mass % or more, and is preferably 70 mass % or less, more preferably 60 mass % or less, even more preferably less than 50 mass %.

The lubricating oil composition of the present invention contains the viscosity index improver of the present invention and a lubricating base oil as essential components and may further contain optional additives and others. For example, the lubricating oil composition preferably further contains at least one additive selected from the group consisting of a pour point depressant, an anti-wear agent, a

metal-base detergent dispersant, an ashless detergent dispersant, an antioxidant, a corrosion inhibitor, an antifoaming agent and a friction modifier.

As the pour point depressant, any pour point depressant used for lubricating oils can be used. Examples of the pour point depressant include, for example, polymethacrylates, naphthalene-chlorinated paraffin condensation products, phenol-chlorinated paraffin condensation products, and others. Among them, polymethacrylates are preferable.

As the anti-wear agent (or an extreme pressure agent), any anti-wear agent or extreme pressure agent used for lubricating oils can be used. As the anti-wear agent (or the extreme pressure agent), a sulfur-base extreme pressure agent, a phosphorus-base extreme pressure agent and sulfur-phosphorus-base extreme pressure agent can be used, for example; and specific examples thereof include zinc dialkyl dithiophosphate (ZnDTP), phosphite esters, thiophosphite esters, dithiophosphite esters, trithiophosphite esters, phosphate esters, thiophosphate esters, dithiophosphate esters, trithiophosphate esters, amine salts of them, metal salts of them, derivatives of them, dithiocarbamate, zinc dithiocarbamate, MoDTC, disulfides, polysulfides, sulfurized olefins, sulfurized greases and others. Among them, sulfur-base extreme pressure agents are preferable, and sulfurized greases are particularly preferable.

Examples of the metal-base detergent dispersant include a normal salt or a basic salt such as an alkali metal/alkaline earth metal sulfonate, an alkali metal/alkaline earth metal phenate, an alkali metal/alkaline earth metal salicylate and others. Examples of the alkali metal include sodium, potassium and others, and examples of the alkaline earth metal include magnesium, calcium, barium and others; and magnesium or calcium is preferable, and calcium is especially preferable.

As the ashless detergent dispersant, any ashless detergent dispersant used in lubricating oils can be used. Examples of the ashless detergent dispersant include, for example, mono- or bis-succinimides having at least one linear or branched alkyl or alkenyl group of 40 to 400 carbon atoms in the molecule, benzylamines having at least one alkyl or alkenyl group of 40 to 400 carbon atoms in the molecule, polyamines having at least one alkyl or alkenyl group of 40 to 400 carbon atoms in the molecule, boron compounds of them, derivatives of them with carboxylic acid, phosphoric acid or the like, and others. In use, one or more kinds arbitrarily selected from these can be blended.

Examples of the antioxidant include ashless antioxidants such as phenolic or amine-base antioxidants and metal-base antioxidants such as copper or molybdenum-base antioxidants. Specific examples of the antioxidant include, for example, phenol-base ashless antioxidants such as 4,4'-methylenebis(2,6-di-tert-butylphenol) and 4,4'-bis(2,6-di-tert-butylphenol), amine-base ashless antioxidants such as phenyl- $\alpha$ -naphthylamine, alkylphenyl- $\alpha$ -naphthylamine and dialkyldiphenylamine, and others.

Examples of the corrosion inhibitor include, for example, benzotriazole compounds, tolyltriazole compounds, thiadiazole compounds, imidazole compound and others.

Examples of the antifoaming agent include, for example, silicone oils having kinematic viscosity at 25°C. of 1,000 to 100,000 mm<sup>2</sup>/s, fluorosilicone oils, alkenylsuccinic acid derivatives, esters of a polyhydroxyaliphatic alcohol and a long-chain fatty acid, methyl salicylate, o-hydroxybenzyl alcohol and others.

Examples of the friction modifier include organic molybdenum compounds such a succinimide molybdenum complex (e.g. molybdenum dithiocarbamate, molybdenum dith-

iophosphate and the like) and an amine salt of an organic molybdcic acid, and compounds having a linear alkyl group of 8 to 30 carbon atoms and a polar group that can be adsorbed on a metal in the molecule. Examples of the polar group include amines, polyamines, amides, amine compounds which simultaneously have these groups in the molecule, fatty acid esters, fatty acid amides, fatty acids, aliphatic alcohols, aliphatic ethers, urea compounds, hydrazide compounds, alkenyl succinimide esters, alcohols or diols, monoalkyl glycerin ester having both an ester and a hydroxyl group, and others. In addition, various compounds such as alkylamine alkoxy alcohols having both an amine group and a hydroxyl group in the molecule are also exemplified.

In the case where the lubricating oil composition contains one or more kinds selected from the group consisting of a pour point depressant, an anti-wear agent, a metal-base detergent dispersant, an ashless detergent dispersant, an antioxidant, a corrosion inhibitor, an antifoaming agent and a friction modifier, the content of each is preferably 0.01 mass % or more and 10 mass % or less, based on the total amount of the lubricating oil composition. In the case where the lubricating oil composition contains an antifoaming agent, the content of that is preferably 0.0001 mass % or more and 0.01 mass % or less. In the case where the lubricating oil composition is used as the base oil composition, the base oil composition may substantially consist of the viscosity index improver and a lubricating base oil, and in this case, the total content of the viscosity index improver and the lubricating base oil is preferably, for example, 98 mass % or more, more preferably 99 mass % or more and even more preferably 99.5 mass % or more, based on the total amount of the base oil composition.

The lubricating oil composition may further contain a viscosity index improver other than the polymer of the present invention, a rust inhibitor, a demulsifier, a metal deactivator and others, in addition to the above components.

The viscosity index improver other than the polymer of the present invention is specifically a non-dispersible or dispersible ester group-containing viscosity index improver, and examples of that include a non-dispersible or dispersible poly(meth)acrylate-base viscosity index improver, a non-dispersible or dispersible olefin-(meth)acrylate copolymer-base viscosity index improver, a styrene-maleic anhydride ester copolymer-base viscosity index improver, mixtures thereof, and others. Among them, a non-dispersible or dispersible poly(meth)acrylate-base viscosity index improver is preferable, and a non-dispersible or dispersible polymethacrylate viscosity index improver is more preferable. Other examples of that include non-dispersible or dispersible ethylene- $\alpha$ -olefin copolymers or hydrides thereof, polyisobutylene or hydrides thereof, styrene-diene hydrogenated copolymers, polyalkylstyrene and others.

Examples of the rust inhibitor include, for example, petroleum sulfonate, alkylbenzene sulfonate, dinonyl naphthalene sulfonate, alkenyl succinate ester, polyhydric alcohol ester and others.

Examples of the demulsifier include, for example, polyalkylene glycol nonionic surfactants such as polyoxyethylene alkyl ether, polyoxyethylene alkyl phenyl ether and polyoxyethylene alkyl naphthyl ether.

Examples of the metal deactivator include, for example, imidazoline, pyrimidine derivatives, alkylthiadiazoles, mercaptobenzothiazole, benzotriazole or derivatives thereof, 1,3,4-thiadiazole polysulfide, 1,3,4-thiadiazolyl-2,5-bisalkyl dithiocarbamate, 2-(alkyldithio)benzimidazole,  $\beta$ -( $\alpha$ -carboxybenzylthio)propionenitrile and others.

This application claims priority to Japanese Patent Application No. 2014-189053, filed on Sep. 17, 2014, and Japanese Patent Application No. 2015-079392, filed on Apr. 8, 2015, and the entire contents of which are incorporated by reference herein.

## EXAMPLES

The present invention will be hereinafter described more specifically by reference to Examples; however, the present invention is not limited to these Examples. In Examples and Comparative Examples, the terms “%” and “parts” respectively represent “mass %” and “part by mass”, unless otherwise noted.

## (1) Analysis Method

## (Weight-Average Molecular Weight and Number-Average Molecular Weight)

Measurement of the weight-average molecular weight and number-average molecular weight of a polymer was conducted by using the following system under the following conditions.

System: GPC system HLC-8220 manufactured by Tosoh Corporation

## Measurement Side Column Configuration

Guard column: TSK guard column Super HZ-L manufactured by Tosoh Corporation

Separation column: TSKgel Super HZM-M 2 columns manufactured by Tosoh Corporation

## Reference Side Column Configuration

Reference column: TSKgel Super H-RC manufactured by Tosoh Corporation

Developing solvent: chloroform (available from Wako Pure Chemical Industries, special grade)

Flow rate of developing solvent: 0.6 mL/min

Standard sample: TSK standard polystyrene (PS-oligomer kit, manufactured by Tosoh Corporation)

Column temperature: 40° C.

## (Branching Degree)

Measurement of the branching degree of a polymer was conducted by using the following system under the following conditions.

System: Viscotek TDA (light scattering/viscosity/refractive index detector) manufactured by Malvern Instruments Ltd was connected to GPC system HLC-8320 manufactured by Tosoh Corporation

## Measurement Side Column Configuration

Guard column: TSKgel guard column H<sub>XZ</sub>-H manufactured by Tosoh Corporation

Separation column: TSKgel GMH<sub>XZ</sub> 2 columns manufactured by Tosoh Corporation

Sample injection amount: 100 µL

Sample concentration: 0.200 mass %

Developing solvent: THF (0.8892 g/mL)

Flow rate of developing solvent: 1.0 mL/min

Equipment calibration sample: TSK standard polystyrene F-10

The branching degree was quantified as follows. A branching degree reference polymer (prepared by the operation described below) and polymers of Examples or Comparative Examples were measured by the above system. Prior to the measurement, a polymer base oil solution of Example or Comparative Example was reprecipitated and dried twice. Reprecipitation was carried out by diluting the polymer with THF to 5 mass % and dropping it in 10 times amount of ethanol with stirring, and drying was carried out

under vacuum at 80° C. for 8 hours. From the measurement results obtained by the above system, Mark-Houwink Plot was prepared using the analysis software OmniSEC (available from Malvern Instruments Ltd). Provided that a straight line, which was obtained by extrapolating a linear region of an absolute molecular weight Mw of 400,000 or less of the branching degree reference polymer having the same composition, corresponds to a straight chain structure, the branching degree of the polymers of Examples or Comparative Examples was calculated using a random polydisperse model. A detailed theory of this is described in the following documents and the description of which is incorporated herein by reference: “GPC School Handbook” (text for workshops), issued by Malvern Instruments Ltd; Hirohide Matsushita, “Polymer Chemistry II Physical Properties”, published by Maruzen Co., Ltd. The branching degree was calculated for the range of the absolute molecular weight Mw of 400,000 to 1,300,000 obtained by the above system.

The branching degree reference polymer was prepared as follows. Into a reaction vessel equipped with a stirrer, a temperature sensor, a cooling tube, a nitrogen inlet tube and a dropping funnel, the same amount of monomers as in the corresponding Example or Comparative Example, 32.3 parts by mass of toluene, 0.05 parts by mass of an antioxidant (ADK STAB (registered trademark) 2112, manufactured by ADEKA Corporation) and 0.05 parts by mass of n-dodecyl mercaptan (DM) as a chain transfer agent were fed, and the content was raised to 105° C. while introducing nitrogen gas thereto. A solution prepared by mixing 0.0258 parts by mass of t-amylperoxyisobornanoate (Luperox 570 (registered trademark), manufactured by Arkema Yoshitomi Ltd.) as a polymerization initiator and 0.46 parts by mass of toluene were added, and solution polymerization was proceeded while dropping a solution prepared by dissolving 0.0258 parts by mass of the polymerization initiator in 2.6 parts by mass of toluene over 1 hour, and then the polymerization was stopped by cooling. The obtained polymerization solution was diluted with THF to 5 mass % and dropping it in 10 times amount of ethanol with stirring. The obtained solid was dried at 80° C. under vacuum for 8 hours to obtain the branching degree reference polymer.

## (Base Oil Solubility)

A base oil solution containing a polymer in the concentration of 30 mass % was judged as A or B according to the following criteria.

A: the solution is transparent, that is visually completely dissolved at 25° C.

B: the solution is cloudy or a residue is visually observed at 25° C.

## (Viscosity Index)

A polymer was diluted with a base oil (viscosity index: 130) so that the kinematic viscosity at 100° C. was 7.0 mm<sup>2</sup>/s, and a viscosity index was measured according to the method of HS K 2283. In the case where the viscosity index was 230 or more, it was judged as A, in the case where the viscosity index was 210 or more and less than 230, it was judged as B, and in the case where the viscosity index was less than 210, it was judged as C.

## (Shear Stability)

A polymer was diluted with a base oil (viscosity index: 130) so that the kinematic viscosity at 100° C. was 7.0 mm<sup>2</sup>/s, and ultrasonic irradiation was applied under the following conditions.

Apparatus: UP400S manufactured by Hielscher Ultrasonics

Setting: Amplitude=70%, Cycle=1

Time: 5 minutes

Temperature: 100° C.

The kinematic viscosity at 100° C. of a base oil and before and after shearing was measured, and in the case where the

value of the SSI was less than 25, it was judged as A, and in the case where the value of the SSI was 25 or more, it was judged as B, wherein the SSI is calculated from the following equation:  $SSI = \{1 - (\text{kinematic viscosity after shearing} - \text{kinematic viscosity of a base oil}) / (\text{kinematic viscosity before shearing} - \text{kinematic viscosity of a base oil})\} \times 100$ .

(SP Value)

The SP value (solubility parameter) of a polymer was calculated using the Materials Studio (registered trademark) Ver. 6.1 MS-Synthia module available from Accelrys AG. First, a monomer structure was created and a repeated structure was defined. Using the defined monomer structure, polymer physical properties such as solubility parameter were calculated with the MS-Synthia module. The MS-Synthia module is a software for calculating physical properties of macromolecules by using Quantitative Structure Property Relationships (QSPR), and by using a bond index obtained from a graph theory, physical properties of macromolecules can be calculated. Detailed theory is described in the following document, and the description of which is incorporated herein by reference: Jozef Bicerano, "Prediction of Polymer Properties, 3rd Edition", published by Marcel Dekker. For this time, among the SP values (solubility parameters) of the Fedors method improved by Bicerano, that is able be calculated by the MS-Synthia, and the van Krevelen method, the value of the Fedors method was employed.

#### (2) Preparation Example of Polymer Base Oil Solution

##### Example 1

Into a reaction vessel equipped with a stirrer, a temperature sensor, a cooling tube, a nitrogen inlet tube and a dropping funnel, 20 parts by mass of methyl methacrylate (MMA), 70 parts by mass of stearyl methacrylate (StMA), 10 parts by mass of N-phenylmaleimide (PMI), 52.8 parts by mass of toluene, 0.05 parts by mass of an antioxidant (ADK STAB (registered trademark) 2112, manufactured by ADEKA Corporation), 0.40 parts by mass of acetic anhydride, 0.05 parts by mass of pentaerythritol tetrakis(mercaptopropionate) were fed, and the content was raised to 105° C. while introducing nitrogen gas thereto. A solution prepared by mixing 0.0258 parts by mass of t-amylperoxyisononanoate (Luperox (registered trademark) 570, manufactured by Arkema Yoshitomi Ltd.) as a polymerization initiator and 0.46 parts by mass of toluene were added, and solution polymerization was proceeded while dropping a solution prepared by dissolving 0.205 parts by mass of the polymerization initiator in 20.5 parts by mass of toluene over 4 hours, and further aging was carried out for 2 hours.

Subsequently, the cooling pipe was replaced by a distilling head connected to a cooling pipe and a distillate receiver, and 233 parts by mass of a base oil (viscosity index 130) was fed into the reaction vessel. After raising a bath temperature to 150° C., the pressure was gradually reduced using a vacuum pump to remove toluene. After 30 minutes from the internal temperature reached 142° C., pressure reduction was released and cooled to obtain a polymer base oil solution (polymer concentration: 30 mass %). The result is shown in Table 1.

##### Example 2

Into a reaction vessel equipped with a stirrer, a temperature sensor, a cooling tube, a nitrogen inlet tube and a

dropping funnel, 35 parts by mass of MMA, 60 parts by mass of StMA, 5 parts by mass of PMI, 32.3 parts by mass of toluene, 0.05 parts by mass of an antioxidant (ADK STAB (registered trademark) 2112, manufactured by ADEKA Corporation), 0.40 parts by mass of acetic anhydride and 0.10 parts by mass of pentaerythritol tetrakis(mercaptopropionate) were fed, and the content was raised to 105° C. while introducing nitrogen gas thereto. A solution prepared by mixing 0.0258 parts by mass of t-amylperoxyisononanoate (Luperox (registered trademark) 570, manufactured by Arkema Yoshitomi Ltd.) as a polymerization initiator and 0.46 parts by mass of toluene was added, and solution polymerization was proceeded while dropping a solution prepared by dissolving 0.205 parts by mass of the polymerization initiator in 20.5 parts by mass of toluene over 4 hours, and further aging was carried out for 2 hours.

Subsequently, the cooling pipe was replaced by a distilling head connected to a cooling pipe and a distillate receiver, and 233 parts by mass of a base oil (viscosity index 130) was fed into the reaction vessel. After raising a bath temperature to 150° C., the pressure was gradually reduced using a vacuum pump to remove toluene. After 30 minutes from the internal temperature reached 142° C., pressure reduction was released and cooled to obtain a polymer base oil solution (polymer concentration: 30 mass %). The result is shown in Table 1.

##### Comparative Example 1

Into a reaction vessel equipped with a stirrer, a temperature sensor, a cooling tube, a nitrogen inlet tube and a dropping funnel, 40 parts by mass of MMA, 60 parts by mass of StMA, 0.05 parts by mass of an antioxidant (ADK STAB (registered trademark) 2112, manufactured by ADEKA Corporation), 0.40 parts by mass of acetic anhydride, 0.10 parts by mass of n-dodecyl mercaptan (DM) and 0.46 parts by mass of toluene were fed, and the content was raised to 105° C. while introducing nitrogen gas thereto. Subsequently, a solution prepared by dissolving 0.205 parts by mass of t-amylperoxyisononanoate (Luperox (registered trademark) 570, manufactured by Arkema Yoshitomi Ltd.) in 10.5 parts by mass of toluene was added dropwise over 4 hours, whereby solution polymerization was proceeded. After thirty minutes from completion of the dropwise addition, 13.5 parts by mass of toluene was added, and further aging was carried out for 2.5 hours.

Subsequently, the cooling pipe was replaced by a distilling head connected to a cooling pipe and a distillate receiver, and 233 parts by mass of a base oil (viscosity index 130) was fed into the reaction vessel. After raising a bath temperature to 150° C., the pressure was gradually reduced using a vacuum pump to remove toluene. After 30 minutes from the internal temperature reached 142° C., pressure reduction was released and cooled to obtain a polymer base oil solution (polymer concentration: 30 mass %). The result is shown in Table 1.

##### Example 3

A polymer base oil solution (polymer concentration: 30 mass %) was obtained in the same manner as in Example 1, except that 70 parts by mass of StMA was replaced by 30 parts by mass of StMA and 40 parts by mass of lauryl methacrylate (LMA). The result is shown in Table 1.

##### Example 4

A polymer base oil solution (polymer concentration: 30 mass %) was obtained in the same manner as in Example 2,

except that 35 parts by mass of MMA was replaced by 20 parts by mass of MMA, 60 parts by mass of StMA was replaced by 30 parts by mass of StMA and 40 parts by mass of LMA, and 5 parts by mass of PMI was replaced by 10 parts by mass of PMI. The result is shown in Table 1.

## Example 5

A polymer base oil solution (polymer concentration: 30 mass %) was obtained in the same manner as in Example 3, except that 0.05 parts by mass of pentaerythritol tetrakis (mercaptoacetate) was replaced by 0.06 parts by mass of hexakis(3-mercaptopropionic acid) dipentaerythritol. The result is shown in Table 1.

## Comparative Example 2

Into a reaction vessel equipped with a stirrer, a temperature sensor, a cooling tube, a nitrogen inlet tube and a dropping funnel, 20 parts by mass of MMA, 30 parts by mass of StMA, 10 parts by mass of PMI, 40 parts by mass of LMA, 32.3 parts by mass of toluene, 0.05 parts by mass of an antioxidant (ADK STAB (registered trademark) 2112, manufactured by ADEKA Corporation), 0.40 parts by mass of acetic anhydride and 0.05 parts by mass of DM were fed, and the content was raised to 105° C. while introducing nitrogen gas thereto. A solution prepared by mixing 0.0258 parts by mass of t-amylperoxyisononanoate (Luperox (registered trademark) 570, manufactured by Arkema Yoshitomi Ltd.) as a polymerization initiator and 0.46 parts by mass of

## Example 6

5  
10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8890  
8895  
8900  
8905  
8910  
8915  
8920  
8925  
8930  
8935  
8940  
8945  
8950  
8955  
8960  
8965  
8970  
8975  
8980  
8985  
8990  
8995  
9000  
9005  
9010  
9015  
9020  
9025  
9030  
9035  
9040  
9045  
9050  
9055  
9060<br

27

The invention claimed is:

1. A viscosity index improver comprising a polymer obtained by polymerizing a maleimide monomer (a) represented by the following formula (1), that is referred to as a "component (a)":



(1)

wherein R<sup>1</sup> and R<sup>2</sup> independently represent a hydrogen atom or an alkyl group, and X represents a hydrogen atom, a linear, cyclic or branched alkyl group, which optionally has an aromatic ring, or an aryl group; an alkyl (meth)acrylate (b) having an aliphatic hydrocarbon group of 6 to 40 carbon atoms, that is referred to as a "component (b)"; and an alkyl (meth)acrylate (c) having an aliphatic hydrocarbon group of 1 to 5 carbon atoms, that is referred to as a "component (c)"; as essential components of a monomer component, in the presence of a tri- or higher functional mercaptan and/or a tri- or higher functional initiator;

wherein

the polymer has a ring structure derived from the component (a) in a main chain, wherein the ring structure is represented by the following formula (4):



(4)

a content of the unit derived from the component (a) is 5 parts by mass or more and 30 parts by mass or less, relative to 100 parts by mass of the polymer, a content of the unit derived from the component (b) is 50 parts by mass or more and less than 95 parts by mass, relative to 100 parts by mass of the polymer, and a content of the unit derived from the component (c) is 2 parts by mass or more and less than 40 parts by mass, relative to 100 parts by mass of the polymer, and

the polymer satisfies the following (1) to (3):

(1) weight-average molecular weight (Mw) of 200,000 or more and 600,000 or less;

(2) number-average molecular weight (Mn) of 90,000 or more;

(3) molecular weight distribution (Mw/Mn) of 4.0 or less.

2. The viscosity index improver according to claim 1, wherein the polymer satisfies the following (4):

(4) branching degree of 1.0 or more.

3. A lubricating oil composition comprising a lubricating base oil and the viscosity index improver according to claim 1, wherein a content of the viscosity index improver is 0.01 mass % or more and 70 mass % or less.

28

4. A viscosity index improver comprising a polymer having a branch unit derived from a tri- or higher functional mercaptan and/or a branch unit derived from a tri- or higher functional initiator, a unit having a ring structure in a main chain of the polymer, wherein the ring structure is represented by the following formula (4):



(4)

wherein R<sup>1</sup> and R<sup>2</sup> independently represent a hydrogen atom or an alkyl group, and X represents a hydrogen atom, a linear, cyclic or branched alkyl group, which optionally has an aromatic ring, or an aryl group, a unit derived from an alkyl (meth)acrylate having an aliphatic hydrocarbon group of 6 to 40 carbon atoms, and a unit derived from an alkyl (meth)acrylate having an aliphatic hydrocarbon group of 1 to 5 carbon atoms, wherein

a content of the unit represented by the formula (4) is 5 parts by mass or more and 30 parts by mass or less, relative to 100 parts by mass of the polymer, a content of the unit derived from an alkyl (meth)acrylate having an aliphatic hydrocarbon group of 6 to 40 carbon atoms is 50 parts by mass or more and less than 95 parts by mass, relative to 100 parts by mass of the polymer, and a content of the unit derived from an alkyl (meth)acrylate having an aliphatic hydrocarbon group of 1 to 5 carbon atoms is 2 parts by mass or more and less than 40 parts by mass, relative to 100 parts by mass of the polymer, and

the polymer satisfies the following (1) to (3):

(1) weight-average molecular weight (Mw) of 200,000 or more and 600,000 or less;

(2) number-average molecular weight (Mn) of 90,000 or more;

(3) molecular weight distribution (Mw/Mn) of 4.0 or less.

5. The viscosity index improver according to claim 4, wherein the polymer satisfies the following (4):

(4) branching degree of 1.0 or more.

6. A lubricating oil composition comprising a lubricating base oil and the viscosity index improver according to claim 4, wherein a content of the viscosity index improver is 0.01 mass % or more and 70 mass % or less.

7. A method for producing a viscosity index improver comprising the step of polymerizing a maleimide monomer (a) represented by the following formula (1), that is referred to as a component (a):



(1)

**29**

wherein R<sup>1</sup> and R<sup>2</sup> independently represent a hydrogen atom or an alkyl group, and X represents a hydrogen atom, a linear, cyclic or branched alkyl group, which optionally has an aromatic ring, or an aryl group; an alkyl (meth)acrylate (b) having an aliphatic hydrocarbon group of 6 to 40 carbon atoms, that is referred to as a “component (b)”; and an alkyl (meth)acrylate (c) having an aliphatic hydrocarbon group of 1 to 5 carbon atoms, that is referred to as a “component (c)”; as essential components of a monomer component, in the presence of a tri- or higher functional mercaptan and/or a tri- or higher functional initiator, thereby obtaining a polymer having a ring structure derived from the component (a) in a main chain,

wherein  
the ring structure is represented by the following formula  
(4):

**30**

a used amount of the component (a) is 5 parts by mass or more and 30 parts by mass or less, relative to 100 parts by mass of the monomer components, a used amount of the component (b) is 50 parts by mass or more and less than 95 parts by mass, relative to 100 parts by mass of the monomer components, and a used amount of the component (c) is 2 parts by mass or more and less than 40 parts by mass, relative to 100 parts by mass of the monomer components.

\* \* \* \* \*